

## UNITED STATES PATENT OFFICE.

JAMES D. KLINGER AND CLETE L. BOYLE, OF DETROIT, MICHIGAN.

## PREPARATION FOR CLEANING METAL PREPARATORY TO PAINTING.

No Drawing.

Application filed December 26, 1925. Serial No. 77,879.

Our invention relates to an improved preparation for cleaning metal, particularly sheet steel, preparatory to painting the metal.

5 The invention concerns itself particularly in the provision of a suitable solvent to be used in conjunction with a rust attacking and removing acid for the removal of rust, oxides, dirt, oils and greases from the surface of sheet steel or metal parts and also from the pores of the metal, in order to satisfactorily clean the same preparatory to painting.

A solvent which we have discovered to be 15 unusually valuable in a solution of this character is known to the chemical art as ethyl methyl ketone or it may be written as methyl ethyl ketone having the formula  $\text{CH}_3\text{COC}_2\text{H}_5$ , or  $\text{C}_4\text{H}_8\text{O}$ .

20 Many different solvents and combinations thereof have been used in conjunction with various rust removing acids for cleaning metal for painting. Solvents such as butyl alcohol, fusel oil, ethyl acetate, mesityl oxide 25 and others have been employed in the art with varying degrees of success. One of the most pronounced objectionable features of these several solvents has been that they must first be blended with ethyl alcohol or 30 acetone to make them miscible with the particular rust removing acid in connection with which they are used, which usually contains a certain percentage of water. Consequently when the cleaning solution is applied to the metal the acetone or ethyl alcohol 35 evaporates, thus throwing the principal solvents out of solution, thereby creating a condition which makes it difficult to satisfactorily rinse all the resultant products of 40 cleaning which contain the solvents that are normally insoluble in water from the surface of the metal. There are, however, certain solvents such as diacetone alcohol and 45 phorone, which when blended with ethyl alcohol seem to prevent the lower boiling point solvents from evaporating, but after blending they lose a certain amount of their solvent properties which lowers their value as cleaning agents.

50 Ethyl methyl ketone possesses the very desirable property of being an excellent solvent for oils and greases, and furthermore, it is miscible alone in an acid solution. Therefore, it can be used in any desired percentage in an acid cleaning solution, the amount used depending upon the prevailing

conditions for cleaning. If evaporation occurs it will only lower the percentage of the ethyl methyl ketone present, and it will not disturb the stability of the solution, with 60 the result that after the cleaning operation is completed the remaining products of cleaning can be readily rinsed from the metal with hot or cold water.

Free or undisturbed rinsing on account of 65 the resultant products of cleaning being rinsed from the pores of the metal as well as from the surface, insures a much cleaner surface over which to paint. Free rinsing, however, is only feasible when all the ingredients used in the cleaning solution are 70 miscible in varying proportions in the metal etching acid used and in water. It is highly important that the resultant products of cleaning be very thoroughly rinsed from the 75 surface of the metal especially if the metal is to be painted with a pyroxylin primer or coated with any pyroxylin material.

In order to produce a satisfactory cleaning solution the ethyl methyl ketone may be 80 blended with a rust removing acid such as phosphoric acid or with a sulphuric acid. A suitable rust inhibiting agent such as a reduced chromium compound may with advantage be added to the admixture. 85

When phosphoric acid is used the solution should be rinsed from the metal with hot water. Phosphoric acid is a syrupy or a sticky acid and great care should be exercised in rinsing in order to remove all of the phosphoric acid from the surface of the metal and also the pores of the metal. By using sulphuric acid and a reduced chromium compound the difficulty of rinsing can be minimized because sulphuric acid has a decided 95 affinity for water and is consequently a free rinsing acid and is readily removable from the pores of the metal as well as from its surface.

When phosphoric acid is employed a satisfactory formula is as follows:

25% by volume 85% ortho phosphoric acid,

35% by volume water,

40% by volume ethyl methyl ketone.

When the sulfuric acid reduce chromium solution is employed a satisfactory formula is as follows:

Dissolve one fourth of a pound of normal sodium chromate in one and one-half quarts 110 of water and add one-half quart of concentrated sulfuric acid. The solution is al-

2  
lowed to cool. It is then reduced with any suitable reducing agent such as a satisfactory carbohydrate until the characteristic bluish green color of reduced chromium compounds 5 predominates. Two quarts of the ethyl methyl ketone are then added to complete the admixture.

This solution may be applied with a brush, sponge or spray to the surface of the 10 metal to be cleaned and after the metal has been cleaned the resultant products of cleaning may be removed therefrom with hot or cold water. When small parts are cleaned they may be dipped or immersed in a tank 15 containing cleaning solution and subsequently dipped in a tank containing the rinse water. After rinsing the metal is dried and is then ready for the priming coat of paint.

In the cases where rapid cleaning of the 20 metal is desired or to lessen the cost of the material used, denatured alcohol may be substituted for a part of the methyl ethyl ketone

in varying amounts. An amount equal to twenty-five per cent by volume of the solution is satisfactory. Denatured alcohol 25 might be employed in a proportion varying from fifteen to thirty-five per cent by volume with fifteen per cent and upwards of the ethyl methyl ketone.

What we claim is:

1. A preparation for cleaning metal for painting, comprising an admixture of phosphoric acid and ethyl methyl ketone in substantially the proportions herein set forth.

2. A preparation for cleaning metal for 35 painting, comprising an admixture of a dilute rust attacking and removing acid, and ethyl methyl ketone in substantially the proportions herein set forth.

In testimony whereof, we sign this specification.

JAMES D. KLINGER.  
CLETE L. BOYLE.